# EUROPEAN PATENT SPECIFICATION

(11) **EP 3 286 342 B1**
(45) Date of publication and mention of the grant of the patent: **28.07.2021**
(21) Application number: 16723529.0
(22) Date of filing: 21.04.2016
(51) Int. Cl.: C14C 3/18, C14C 3/20, C14C 3/22, C14C 3/28, C14C 3/16, C14C 9/02

(54) **SKINS TANNING PROCESS**
GERBVERFAHREN FÜR HÄUTE
PROCÉDÉ DE TANNAGE DE PEAUX

(30) Priority: 21.04.2015 IT TV20150055
(43) Date of publication of application: 28.02.2018
(73) Proprietor: Osmo S.r.l., 36071 Arzignano (IT)
(72) Inventor: NICOLETTI, Fabrizio, 36071 Arzignano (IT); PIAZZA, Andrea, 36071 Arzignano (IT); MASSIGNAN, Ludovico, 36071 Arzignano (IT)
(74) Representative: Cernuzzi, Daniele
(86) International application number: PCT/IB2016/052282
(87) International publication number: WO 2016/170503

(56) References cited:
- EP-B1- 1 831 405
- US-A- 4 245 996
- US-A1- 2007 294 836

## Description

### TECHNICAL FIELD

The present invention relates to a skins tanning process.

### BACKGROUND ART

Skins tanning, i.e. the processing undergone by animal skins to turn them into leather, in an ancient process, but nowadays it is carried out with advanced techniques.

Generally speaking, a tanning process includes preliminary operations producing the so-called pelt; the actual tanning; the retanning; and dressing treatments.

Preliminary operations are basically aimed at removing, from the skins, various impurities and the preservatives used to maintain the skins intact until the tanning process as well as at restoring the features of the skins, thus making them suitable for the following actual tanning treatments.

Then, tanning transforms the pelt into leather by means of proper tanning substances, which penetrate the skin and are steadily fixed to the dermal fibres. There are different types of tanning (vegetable tanning, mineral tanning, etc.), which differ from one another because of the tanning substances used and of the ways in which these substances are applied; some types of tanning are better than others for the treatment of certain skins and, generally speaking, manufacturers select the tanning process that is deemed to be the most appropriate to obtain specific features of the end product.

After the actual tanning there is a retanning step, which is used to define the specific features of the skins depending on the article to be manufactured; the skins are then subjected to dressing operations, even based on the uses for which the skins are intended.

US4245996A discloses sulphonated condensation products based on naphtalene and phenol and which are used as tanning agents for the production of leather and as re-tanning agents for re-tanning mineral-tanned leather.

Tanning processes known at the moment have proven to be not good enough, in particular from the point of view of their environmental impact. As a matter of fact, known processes, because of the products used in the different processing steps and of the techniques involved, cause the production of waste waters and of processing waste that are highly polluting and, anyway, are very difficult to be handled from an environmental point of view; moreover, they do not lead to an end product or to a processing waste that are completely (or at least largely) biodegradable or compostable.

### DISCLOSURE OF INVENTION

The object of the present invention is to provide a tanning process that is not affected by the above-mentioned drawbacks shown by prior art processes; in particular, it is an object of the present invention to provide a tanning process that allows manufacturers to obtain a fully biodegradable product, besides being versatile and effective, which leads to the production of high-quality products.

Therefore, the present invention relates to a tanning process as defined, in its essential aspects, in appended claim 1 and, in its additional features, in the dependent claims.

The process according to the present invention, thanks to the specific products used and to the processing techniques applied, allows manufacturers to obtain a fully biodegradable product.

Furthermore, the process according to the present invention allows the skins to gain (after having been dried) features that are comparable with the ones obtained with traditional techniques, in particular softness, a peasant feel, colouring and technical performances that are suitable for the use in different fields, such as shoes, leather products, furniture, car upholstery, etc.

### BRIEF DESCRIPTION OF THE DRAWINGS

Further features and advantages of the invention will be best understood upon perusal of the description of the following non-limiting embodiments, with reference to the accompanying figures, wherein:
- figure 1 contains a table (Table I) showing examples of the ways in which a preliminary step, in particular a soaking-liming step, of the process according to the invention can be carried out;
- figure 2 contains a table (Table II) showing examples of the ways in which further steps, defining - as a whole - a tanning macro-step, of the process according to the invention can be carried out;
- figure 3 contains a table (Table III) showing examples of the ways in which a retanning step of the process according to the invention can be carried out.

### BEST MODE FOR CARRYING OUT THE INVENTION

The process according to the invention is advantageously carried out in drums, for example in the ways (processing recipes) shown, by way of example, in the appended tables.

Advantageously, all operations are carried out in a rotary drum, which is manually or semi-manually operated or is controlled by a control unit, which automatically manages, based on operating schedules corresponding to pre-set recipes, the operation of the drum and, therefore, the different steps of the process.

For example, the drum can be set so as to rotate for predetermined time intervals at the desired speed, if necessary alternating rest times (still drum).

In the appended tables, an indication such as "automatic cycle x-y-x" indicates that the drum rotates for periods of x minutes alternated with rest periods of y minutes.

Obviously, the indications provided below and contained in the appended tables must be interpreted as merely explanatory and the operating modes of the process, in particular the products used, their quantity and the duration of the single operations and steps, can be different from the ones shown.

The drum is drained, when the processing recipe requires to do so, through suitable openings.

The process according to the present invention is used to treat raw skins, for example skins that are freshly salted immediately after having flayed the animal.

Raw skins are firstly introduced into the drum for a preliminary soaking-liming step, during which, in substantially known ways, the first processing in preparation of the tanning is carried out, thus obtaining the so-called pelt (state of the skin at the end of the preliminary soaking-liming step).

By mere way of example, the preliminary step is carried out in the ways shown in appended Table I of figure 1 where the compositions of the products used are indicated as percentage of the weight of the raw skin treated in the preliminary step.

Here and below and in all tables, the commercial names of the products used are provided by mere way of example; each product indicated herein can be replaced with equivalent products.

Then, there is a tanning macro-step carried out, for example, in the ways shown in Table II of figure 2, which comprises four main steps: deliming, bating, pickling, tanning.

In Table II and in the description below, the compositions of the products used in the tanning macro-step are indicated as percentage of the weight of the pelt of the skin i.e. of the weight of the material obtained from the preliminary step and destined to the tanning macro-step.

The deliming step has the function of completely removing the lime absorbed by the skin during the preliminary soaking-liming step.

According to the invention, it is important that the lime is completely removed.

In the deliming step, at first, a first bath is used, which contains:
- 50-100% cold water;
- 0.1-0.5% ammonium sulfate;
- 0.1-1.0% thioglycolic acid (e.g.: COSMOCAL E).

The drum is caused to rotate for 15-45 minutes, then it is drained.

Subsequently, after having drained the drum, (cold) water is added, in particular 30-100%; then, in successive stages, a deliming agent is added, in particular a sulfamic acid-based deliming agent (e.g.: DECALCINANTE A-OS SPECIAL), in increasing quantities:
- 0.5-2.0%, preferably approximately 1.0%, rotating for 15-45 minutes (for example, 30 minutes);
- 0.5-3.0%, preferably approximately 1.5%, rotating for 15-45 minutes (for example, 30 minutes);
- 1.0-5.0%, preferably approximately 3.0%, rotating for 120-240 minutes (for example, 180 minutes);

The drum is drained and a delimed skin is obtained, which is completely free from lime.

After having been delimed, the skin undergoes a bating treatment, which basically consists in the removal of the so-called surface shield (residues of proteins, albumins, etc.) and of elastin. The bating step can be carried out in basically known ways, through suitable degreasing substances and enzymes as indicated, for example, in Table II.

Subsequently, the skin is subjected to a pickling step, consisting in conditioning the skin at a highly acid pH below 4 and approximately ranging from 2.7 to 3.5, preferably around 3-3.2.

The pickling step is carried out with known products, basically, sodium chloride, formic acid and sulfuric acid, but, according to the invention, it requires specific operating techniques, which ensure a particular balance among the content of water, salts and acids in the treatment bath contained in the drum, this condition being necessary to make sure that the subsequent addition of the tanning substance and the penetration into the section of the skin produce good results.

The pickling step is carried out as follows:
After having emptied the drum from the water left by the previous bating step, the drum is filled with a bath containing:
- 20-30% cold water;
- 4-10% sodium chloride;
- 0.3-0.7% sodium formate.

The drum is caused to rotate for 10-20 minutes and then density of the bath is controlled to make sure that it ranges from 8 to 10 degrees Baumé.

Then there is the addition of:
- 1% formic acid at 85%, rotating for 30-60 minutes;
- 1% sulfuric acid at 98%, rotating for 3-4 hours.

This is followed by a rest step lasting 12-24 hours, during which the drum rotates, for example, with cycles of 5-10 minutes alternated with pauses of 60-90 minutes.

The result is a bath with a pH below 4 and approximately ranging from 2.7 to 3.5, preferably ranging from approximately 3 to 3.2.

The total content of water at the end of the pickling step (hence, before the tanning step), starting from 25% of initial water and after the addition of the diluted acids, is approximately 40% +/- 5%.

In any case, it is important to remember that the content of water at the beginning of the tanning step should range from 25% to 55%. As a matter of fact, experiments have shown that a total water content below 25% or exceeding 55% slows down - or even completely blocks - the penetration of the tanning product and, therefore, the stability of the tanning itself.

Then there is the actual tanning step, during which a tanning product (2-10%) is added to the drum, which contains an acid naphthalene tannin, an acid phenolic tannin and sodium sulphate; and a synthetic ester (0.1-1.0%). The drum is rotated for 5 hours.

At the end of the tanning step, the skins are discharged from the drum without being washed (contrary to what normally happens in traditional tanning processes).

This type of tanning allows manufacturers to obtain a partial stabilization of the skins, which can be stored after having been subjected to pressing or, if necessary, complete drying, split, shaved and, at the end, sent to the retanning and drying steps.

Once the skins have been split and/or shaved to obtain the desired thickness, they are reintroduced into drums, in which a retanning step is carried out so as to give to the skins, after the drying thereof, high softness, a peasant feel, colouring and technical performances that are useful in the production of articles such as shoes, leather products, furniture, car upholstery, etc.

The retanning step is carried out, for example, in the ways shown in Table III of figure 3, where, like in the description below, the compositions of the products used are indicated as percentage of the weight of the shaved skin (material ready for the retanning step).

In particular, the retanning step is carried out using a retanning compound containing a C4-C6 linear di-aldehyde in an aqueous solution, wherein the di-aldehyde is available in quantity ranging from 1 to 15% of the weight of the treated skin.

For example, the retanning compound is prepared by mixing, for example, through rotation in the drum for approximately 20 minutes:
- 150-250% hot water (at 40°);
- 1-15% of a C4-C6 linear di-aldehyde in an aqueous solution (e.g.: COSMOWHITE 58).

Then the skins are introduced into the drum, which is rotated for 60 minutes.

Subsequently, a fatliquor (8-12%) is added, for example a synthetic oil mixed with deodorized sulphited fish oil (e.g.: COSMOFAT G), rotating for 30 minutes; then a liquid tanning product (8-12%) is added, which contains sulphone-based synthetic tannins, in particular phenolsulphone-based and/or di-idroxy-diphenilsulphonebased (e.g.: COSMOWHITE SR), rotating for 120 minutes.

Then the drum is rotated for periods of 3 minutes with rest intervals of 30 minutes for a whole night (8 hours).

The drum is drained and two washing steps are carried out with 300% of hot water (40°C).

Then a bath of 100% hot water (40°C) is added, as well as a metal-free colouring agent, rotating for 30 minutes.

Subsequently, there is the addition of:
- 15-25% of a vegetable fatliquor, for example a vegetable lecithin-based one (e.g.: COSMOFAT C), rotating for 30 minutes;
- 5-15% of an acrylic resin at 25% (e.g.: COSMOWHITE H), rotating for 30 minutes;
- 5-15% of a vegetable extract-base filler (e.g.: COSMOWHITE F), rotating for 120 minutes;
- 2-3% of formic acid, rotating for 30 minutes;
- 2-3% of formic acid, rotating for 30 minutes;
- 5-15% of the tanning product containing sulphone-based synthetic tannins (e.g.: COSMOWHITE SR), rotating for 120 minutes.

The drum is drained and two further washing steps are carried out.

Subsequently, the skin is pressed, vacuum-dried at a temperature not exceeding 40°C and then hung in a catenary for complete drying.

Once the skin has dried, it can be processed to manufacture any kind of article.

The products used for the dressing of the skins must be selected so as not to jeopardize the biodegradability of the leather obtained with the process according to the invention.

The process described and explained herein can be subjected to further changes and variants, which do not go beyond the scope of protection of the appended claims.

## Claims

1. Tanning process, comprising a tanning step and a retanning step; the process being **characterized in that** the tanning step comprises the steps of: treating skins in a drum with a bath containing a tanning product comprising an acid naphthalene tannin, an acid phenolic tannin and sodium sulphate; and optionally a synthetic ester; and the retanning step comprises the steps of: treating the skins in a drum with a retanning bath containing an aqueous solution of a di-aldehyde, in particular a C4-C6 linear di-aldehyde; adding a fatliquor; adding a liquid tanning product containing sulphone-based synthetic tannins, in particular phenolsulphone-based and/or di-idroxy-diphenilsulphonebased; adding a vegetal-base filler.

2. A process according to claim 1, wherein the retanning step comprises then the further steps of: draining the drum; effecting at least one and preferably two washes with water; optionally adding a coloring bath; adding a vegetal-base fatliquor; adding an acrylic resin; adding a vegetal-base filler; adding formic acid, in one or more times; adding a tanning product containing sulphone-base synthetic tannins; draining the drum; effecting at least one and preferably two more washes with water.

3. A process according to claim 1 or 2, wherein at the end of the tanning step the skins are discharged from the drum without being washed for being then subjected to the retanning step.

4. A process according to one of the preceding claims, comprising, before the tanning step, a step of deliming, performed so as to remove completely the lime that the skins have absorbed previously, in particular in a preliminary step of soaking-liming.

5. A process according to one of the preceding claims, comprising, before the tanning step, a pickling step, comprising the steps of: treating the skins in a drum with a bath containing sodium chloride and sodium formate, the bath having a density ranging between 8 and 10 degrees Baumé; adding formic acid; adding sulfuric acid, for obtaining a bath having a pH lower than 4 and ranging between 2,7 and 3,5 and preferably ranging between 3,0 and 3,2.

6. A process according to one of the preceding claims, wherein the total water content at the end of the pickling step and before the tanning step is comprised between 25% and 55% of the pelt weight of the skins treated.

7. Tanned skin, i.e. leather, **characterized by** being obtained by the tanning process according to one of the preceding claims.

## Patentansprüche

1. Gerbverfahren, das einen Gerbungsschritt und einen Nachgerbungsschritt umfasst; wobei das Verfahren **dadurch gekennzeichnet ist, dass** der Gerbungsschritt die folgenden Schritte umfasst: Behandeln von Häuten in einer Trommel mit einem Bad, das ein Gerbprodukt enthält, das ein saures Naphthalintannin, ein saures Phenoltannin und Natriumsulfat; und optional ein synthetisches Ester umfasst; und der Nachgerbungsschritt die folgenden Schritte umfasst: Behandeln der Häute in einer Trommel mit einem Nachgerbungsbad, das eine wässrige Lösung eines Dialdehyds, insbesondere eines linearen C4-C6-Dialdehyds, enthält; Beimengen eines Fettlickers; Beimengen eines flüssigen Gerbprodukts, das synthetische Tannine auf Sulfonbasis, insbesondere auf Phenolsulfonbasis und/oder Dihydroxy-Diphenylsulfonbasis enthält; Beimengen eines Füllstoffs auf pflanzlicher Basis.

2. Verfahren nach Anspruch 1, wobei der Nachgerbungsschritt dann die folgenden weiteren Schritte umfasst: Entleeren der Trommel; Durchführen mindestens einer und vorzugsweise zweier Wäschen mit Wasser; optional Beimengen eines Färbungsbades; Beimengen eines Fettlickers auf pflanzlicher Basis; Beimengen eines Acrylharzes; Beimengen eines Füllstoffs auf pflanzlicher Basis; ein- oder mehrmaliges Beimengen von Ameisensäure; Beimengen eines Gerbprodukts, das synthetische Tannine auf Sulfonbasis enthält, Entleeren der Trommel; Durchführen mindestens einer und vorzugsweise zweier oder mehr Wäschen mit Wasser.

3. Verfahren nach Anspruch 1 oder 2, wobei am Ende des Gerbungsschritts die Häute aus der Trommel entnommen werden, ohne gewaschen zu werden, sodass sie dann dem Nachgerbungsschritt unterzogen werden.

4. Verfahren nach einem der vorhergehenden Ansprüche, das vor dem Gerbungsschritt einen Schritt des Entkalkens umfasst, der so durchgeführt wird, dass der Kalk, den die Häute vorhergehend, insbesondere in einem vorbereitenden Schritt des Einweichens-Kalkens, absorbiert haben, vollständig entfernt wird.

5. Verfahren nach einem der vorhergehenden Ansprüche, das vor dem Gerbungsschritt einen Beizschritt umfasst, der die folgenden Schritte umfasst: Behandeln der Häute in einer Trommel mit einem Bad, das Natriumchlorid und Natriumformiat enthält, wobei das Bad eine Dichte aufweist, die zwischen 8 und 10 Grad Baumé beträgt; Beimengen von Ameisensäure; Beimengen von Schwefelsäure zum Erhalten eines Bades, das einen pH-Wert aufweist, der niedriger als 4 ist und zwischen 2,7 und 3,5 beträgt und vorzugsweise zwischen 3,0 und 3,2 beträgt.

6. Verfahren nach einem der vorhergehenden Ansprüche, wobei der Gesamtwassergehalt am Ende des Beizschritts und vor dem Gerbungsschritt zwischen 25 % und 55 % des Blößengewichts der behandelten Häute beträgt.

7. Gegerbte Haut, d. h. Leder, **dadurch gekennzeichnet, dass** sie durch das Gerbverfahren nach einem der vorhergehenden Ansprüche erhalten wurde.

## Revendications

1. Procédé de tannage, comprenant une étape de tannage et une étape de retannage ; le procédé étant **caractérisé en ce que** l'étape de tannage comprend les étapes de : traitement de peaux dans un tambour avec un bain contenant un produit de tannage comprenant un tannin naphtalène acide, un tannin phénolique acide et du sulfate de sodium ; et éventuellement un ester synthétique ; et l'étape de retannage comprend les étapes de : traitement des peaux dans un tambour avec un bain de retannage contenant une solution aqueuse d'un dialdéhyde, en particulier d'un dialdéhyde linéaire en C4 à C6 ; addition d'une liqueur grasse ; addition d'un produit de tannage liquide contenant des tannins synthétiques à base de sulfone, en particulier à base de phénol-sulfone et/ou de dihydroxydiphénylsulfone ; addition d'une charge d'origine végétale.

2. Procédé selon la revendication 1, dans lequel l'étape de retannage comprend ensuite les étapes ultérieures de : drainage du tambour ; réalisation d'au moins un et de préférence deux lavages à l'eau ; éventuellement addition d'un bain colorant ; addition d'une liqueur grasse à base végétale ; addition d'une résine acrylique ; addition d'une charge à base végétale ; addition d'acide formique, en une ou plusieurs fois ; addition d'un produit de tannage contenant des tannins synthétiques à base de sulfone ; drainage du tambour ; réalisation d'au moins un et de préférence deux lavages à l'eau.

3. Procédé selon la revendication 1 ou 2, dans lequel, à la fin de l'étape de tannage, les peaux sont déchargées du tambour sans être lavées pour être ensuite soumises à l'étape de retannage.

4. Procédé selon l'une des revendications précédentes, comprenant, avant l'étape de tannage, une étape de déchaulage, réalisée de manière à éliminer complètement la chaux que les peaux ont absorbée antérieurement, en particulier dans une étape préliminaire de trempage-chaulage.

5. Procédé selon l'une des revendications précédentes, comprenant, avant l'étape de tannage, une étape de piclage, comprenant les étapes de : traitement des peaux dans un tambour avec un bain contenant du chlorure de sodium et du formiate de sodium, le bain ayant une densité s'établissant entre 8 et 10 degrés Baumé ; addition d'acide formique ; addition d'acide sulfurique, pour l'obtention d'un bain ayant un pH inférieur à 4 et s'établissant entre 2,7 et 3,5, et de préférence s'établissant entre 3,0 et 3,2.

6. Procédé selon l'une des revendications précédentes, dans lequel la teneur totale en eau à la fin de l'étape de piclage et avant l'étape de tannage est comprise entre 25 % et 55 % du poids en peau des peaux traitées.

7. Peau tannée, c'est-à-dire cuir, **caractérisée en ce qu'**elle est obtenue par le procédé de tannage selon l'une des revendications précédentes.
